

June 20, 1933.

J. A. BOYER ET AL

1,914,939

NONMETALLIC RESISTOR AND METHOD OF MAKING THE SAME

Filed Dec. 9, 1930



*Fig.2.*



*Fig.3.*



*Fig.4.*



John A. Boyer  
Alma J. Thompson  
By their attorney  
Byrne, Bitter, Pamela, Inc.

## UNITED STATES PATENT OFFICE

JOHN A. BOYER AND ALMER J. THOMPSON, OF NIAGARA FALLS, NEW YORK, ASSIGNEES  
TO GLOBAR CORPORATION, OF NIAGARA FALLS, NEW YORK, A CORPORATION OF NEW YORK

## NONMETALLIC RESISTOR AND METHOD OF MAKING THE SAME

Application filed December 9, 1930. Serial No. 501,020.

This invention relates to improvements in non-metallic resistors made from silicon carbide, and to improved methods in their manufacture. The invention has for its object the 5 production of an element with improved electrical properties.

Silicon carbide resistors are well known in the art of electric heating, and possess the advantage that they may be operated at 10 temperatures up to 1400° C. without protection from the atmosphere. However, the electrical properties of these elements as made by the usual processes are not as satisfactory as might be desired. The resistors usually 15 have the undesired property of greatly decreasing in resistance with rising temperature, so that as the temperature of the resistor increases, the power input at constant voltage also increases. It will be evident that, 20 unless the operating voltage is carefully regulated, a cumulative cycle will obtain wherein the rise in temperature will cause an increase in the power consumed by the element, and the increased power will cause an additional 25 rise in temperature, until the resistor is heated to a temperature much beyond that which it will withstand.

The action may be very rapid when once begun, and instances have been known where 30 the resistor has actually "exploded" from the sudden increase in current, the pieces of the element being scattered with considerable violence.

With silicon carbide elements made by our 35 improved process, the temperature coefficient of electrical resistance becomes markedly positive before the maximum safe temperature of operation of the element is reached. Thus as the temperature of the element approaches that at which rapid oxidation takes place, the current at constant voltage, instead of being increased, is considerably decreased. The strongly positive 40 temperature coefficient affords the additional 45 advantage that the power input is to a certain degree automatically regulated by variations in the temperature of the furnace. As an example, if the furnace is suddenly cooled by the introduction of a cold charge, the elements will decrease in resistance and addi-

tional current will be supplied over that which normally obtains at a somewhat higher temperature.

It is known that if silicon carbide resistors are manufactured by the process of 55 self-bonding or recrystallization, the temperature coefficient of resistance is in some cases slightly positive at temperatures above 700-800° C. However, the order of magnitude of this effect has heretofore been small 60 and magnitude and range of positive temperature coefficient has not been subject to control. The increase in resistance with temperature becomes less as the element is used, and the coefficient may even change in sign 65 and become negative during the life of the resistor.

In making our resistors, we have found that there is a relationship between the type 70 of grain employed and the magnitude of the resistance-temperature coefficient obtained. By using a comparatively pure grain, as for example one that analyzes 99 to 99.5 percent silicon carbide, we have been able to obtain consistently, elements which show an increase 75 in resistance with rise in temperature of thirty to forty percent at temperatures above 700°-800° C.

As an example of a method which may be 80 employed, in making our resistors, we prepare a mix of substantially pure silicon carbide grain, to which is added temporary bonding material such as sodium silicate. The elements are then formed into the desired shape 85 by a suitable compacting process such as tamping. After forming, it is desirable to give the resistors a preliminary baking at approximately 600° C. in order to afford greater mechanical strength for handling. The elements may then be cured by embedding 90 them in a mixture of sand and carbon and passing an electric current through the resistor itself for a predetermined period of time.

In obtaining a substantially pure grain for 95 the preparation of the mix, it is possible in some cases to select silicon carbide as it comes from the furnace so that the grade will be suitable. This is especially true if pure materials are used in making the silicon car- 100

bide. The green variety of silicon carbide, which varies from a dark green to a practically colorless or transparent grain, is more suitable than black silicon carbide when no 5 subsequent purification treatments are used. With grain which is purified by methods which will be hereinafter described, the so-called "run-of-mill" grain may be used. This grain will usually analyze about 95 to 96 percent silicon carbide before subjection to the 10 purification treatment.

In order to purify the grain, the crude lump silicon carbide as it comes from the furnace is crushed and is then treated with a suitable 15 acid which will remove a considerable portion of the surface impurities. As an example, dilute or moderately concentrated sulphuric acid can be used. For further purification, the grain can be subjected to an additional treatment with a solution of an alkali, such as sodium hydroxide. The impurities contained in the silicon carbide are largely 20 on the surface of the grains, and these impurities are to a large extent removed by acid and alkali washing. A grain which is both acid and alkali washed will analyze approximately from 99 to 99.5 percent silicon 25 carbide.

The burning bed which we prefer to use 30 for curing our resistors, and the effect of purifying the silicon carbide grain on the electrical properties of the elements so produced, is shown in the accompanying drawing.

35 In the drawing:

Figure 1 shows a burning bed which may 40 be used for curing the resistors;

Figure 2 shows the change in specific resistance with temperature of two representative elements made from acid and alkali washed grain, the mix containing 32.5 percent 45 120 mesh silicon carbide, 65 percent 280 mesh silicon carbide and 2.5 percent carbon;

Figure 3 shows the effect of acid washing 50 the grain upon the resistance temperature characteristics of the resulting resistor, curve C showing the variation of the specific resistance with temperature of a resistor made from an impure untreated grain, and curve D 55 the variation in specific resistance with temperature of a resistor made from the grain after it has been boiled with sulphuric acid to remove a considerable portion of the surface impurities; and

Figure 4 shows the effect of alkali washing 60 subsequent to an acid washing treatment, curve E showing the variation of the specific resistance with temperature of a resistor made from grain which has been acid washed only, and curve F the variation of the specific 65 resistance with temperature of a resistor made from the same grain as in curve E except that it has been subjected to an additional treatment with boiling sodium hydroxide solution.

The grain, which has been purified as above described, is classified according to grit sizes, and is made into a mix which will give the desired electrical resistance to the finished element. As an example of a mix which may 70 be used, the following is given:

|                                                         | Per cent |
|---------------------------------------------------------|----------|
| 120 mesh silicon carbide, acid and alkali washed        | 32.5     |
| 280 mesh silicon carbide powder, acid and alkali washed | 65       |
| Carbon (lamp black)                                     | 2.5      |

The resistance-temperature characteristics of typical elements made from the above mix are shown in Figure 2. The minimum resistance which the element attains between 0° and 1500° C. is approximately two-thirds the resistance at room temperature, and the increase in resistance through the range in which the temperature coefficient is positive is from 30 to 40 per cent. The electrical resistance of the finished element and the resistance-temperature coefficient are both dependent upon the manner of burning and the 85 temperature and duration of heating during the curing process.

In the preferred method of curing the resistor, it is desirable to mix the grain with a 90 temporary binding agent such as sodium silicate, and to give the formed article a preliminary baking at approximately 600° C., before removal from the mold in order to afford additional strength for handling. The resistors are then removed from the mold, and 95 are dipped in a slip or slurry containing fine sand, carbon and water, the sand and carbon, being in approximately the proportion of 66 1/2 parts of sand to 33 1/2 parts of carbon. The elements are then placed in a burning 100 furnace of the type shown in Figure 1, which consists of a refractory bottom or trough 1, with electrodes at either end for conducting the current. The refractory bottom is covered to a depth of about two inches with a 105 mixture 3 of fine silica and carbon, in the proportion of three parts of silica to one part of carbon.

The coated resistors 4 are then placed carefully upon the bedding material described 110 above in end-to-end relationship extending from one electrode to the other and electrically joined to each other and to the electrode by means of graphite blocks 5 and a paste 6 comprising graphite, silicon and  $Na_2SiO_4$ — 115 (50—50) 0 grade 42.5° gravity. When the rods have been laid down and joined to form a continuous path for the current they are covered with a silica and carbon mixture similar to that used for the bottom or bedding 120 mix and are ready then for burning or curing. Burning or curing is then effected by applying current to the electrodes 2.

It will be seen from Figure 1 and from the 125 above description that the resistors are so 130

positioned in the furnace that their longitudinal axes lie within the path taken by the current in traversing the furnace from electrode to electrode and that their axes coincide with the axis of the path of the heating current. In fact the resistors carry most of the current after the first few minutes of the burning.

Because of the resistance of the uncured 10 resistor, a voltage of approximately 500 volts per linear foot of furnace charge between electrodes may be required at the start to send sufficient current through the furnace to heat up the bedding material and the resistors. 15 However, as the resistors approach the maximum temperature they approach the normal resistance for which they were designed and the applied voltage is cut down to avoid further substantial change. For example, a 20 furnace load six feet long, comprising resistors designed to operate at 110 volts per linear foot may require approximately six times 110 volts for the final applied voltage, but at the start will require approximately 25 six times 500 volts to force the heating current through the furnace.

Resistors of different cross-sectional areas require different current values for the production and maintenance of the maximum 30 temperature and also require maintenance of the maximum temperature for somewhat different periods of time. Obviously resistors of large cross-sectional area require higher current values for the production of 35 maximum temperatures than do smaller resistors of the same general nature. It may be stated, however, by way of example, that a rod of circular cross-section approximately  $\frac{1}{2}$  inch in diameter will require approximately 40 4 kw. per foot for a total time of approximately 8 minutes.

The temperature of the process is believed to be between approximately 2000 and 2200° C., although exact measurement is difficult, 45 owing to the fact that the material must be covered, and that more or less opaque fumes are evolved which interfere with the optical pyrometer readings. It is not necessary to regulate the temperature directly, since the 50 temperature is usually controlled by regulating either the power input or amperage, the proper current being determined experimentally for a given diameter of element and a given amount of covering material. It 55 has been found that the conditions above stated, 4 kw. per ft. for 8 minutes with a  $\frac{1}{2}$  inch diameter element, will produce a satisfactory resistor.

In the method of curing described above, 60 the crystalline particles composing the resistor are bonded by a process usually known as "recrystallization". In this process no permanent binding material is used, the sodium silicate originally present as a temporary binder being decomposed at the tem-

perature of curing. In the process of recrystallization, the article is heated to a temperature where vaporization of the silicon carbide takes place, and the particles grow together, presumably by evaporation and re-deposition, until a strong coherent mass is obtained. In such cases it is generally presumed that the large particles grow at the expense of the small ones.

While the actual mechanism involved in obtaining a strongly positive temperature coefficient at the operating temperature by the use of pure grain is not completely understood, it is believed to be caused by a reduction in the contact resistance at the surface of the various particles making up the resistor.

In a self-bonded resistor made by recrystallization there is apparently a relationship between the conductivity of the element and the magnitude of the positive temperature coefficient. Any factor which tends to increase the contact resistance between particles (as for example, oxidation of the resistor during use, or the introduction of non-metallic or non-conducting materials into the mix) either decreases the positive temperature coefficient or causes the coefficient to become negative throughout the entire range of temperature.

The effect of the acid washing treatment is shown in Figure 3. Curve C shows the change in resistance with temperature of a comparatively impure grain, analyzing 95.5% silicon carbide. Curve D shows the change in resistance with temperature of the same grain which has been subjected to an acid treatment, and has a purity of approximately 98.5 percent. The conductivity of the element is increased approximately ten times, and the temperature coefficient changes from negative throughout the entire range to positive between 750° and 1500° C., the increase in resistance in this range with rising temperature being approximately 20 percent.

There are certain variations in the process of manufacture of a silicon carbide resistor which permit a still further control of the temperature coefficient of resistance. We have found that the grit sizes employed in the resistor mix influence to a certain degree the resistance-temperature characteristics of the resulting element. If a considerable quantity of fine powder is used, as for example 50 to 80 percent of a grit size between 200 and 300 mesh, and if the grain employed is substantially pure silicon carbide, as for example an acid and alkali washed material, an element having a very positive resistance temperature characteristic can be obtained. The reason for the effect produced by using fine powders is not definitely known. However, we believe that the powder either offers a greater surface for contact between the inter-granular particles, or evaporates and recrystallizes much more readily during the cur-

ing process than is the case with coarser crystals.

As shown by the curves and drawing, the resistors made by our improved process have a negative coefficient of resistance up to a dark red heat, above which, however, this coefficient becomes positive. A negative temperature coefficient at low temperatures is characteristic of any silicon carbide resistor known at the present time. With our improved elements the magnitude of the negative temperature coefficient has been considerably decreased over that which obtains with the usual silicon carbide heating element.

The presence of a strongly negative coefficient in the lower temperature range has always been a decided disadvantage, since it greatly decreases the rate of heating. With the usual silicon carbide resistor, the cold resistance is usually so high that the initial current which flows when the element is first placed in the circuit is not sufficient to cause rapid heating. This factor has been a great disadvantage for many applications where speed of heating is important, such as when the element is used in hot plates or stove units. As an example, in the use of a hot plate for boiling water, the total time necessary usually does not exceed fifteen minutes, and with the usual silicon carbide resistor a considerable portion of this time may be consumed in merely bringing the resistor to the operating temperature.

With our improved elements the cold resistance is approximately only one and a half times the resistance at the operating temperature, whereas with the usual silicon carbide resistor the cold resistance is from two to three times the resistance at the operating temperature. In our resistors the initial current is increased from 50 to 100 percent over that which obtains with the usual element having the same ampere rating at the temperature of operation. Such an increase in the initial current has a much greater effect on the rapidity of heating than the magnitude of the resistance indicates, since the time necessary for heating is increased several times for even a comparatively small decrease in the initial current. The term "resistor" as herein used means a resistor adaptable for operation as an electric heating element.

We claim:

1. A recrystallized silicon carbide resistor made from grain of a purity greater than 99 percent.

2. A silicon carbide resistor comprising a recrystallized mass of silicon carbide grains, which grains have been cleaned of those surface impurities which form on silicon carbide in the manufacture thereof.

3. A silicon carbide resistor having a positive temperature coefficient of resistance formed from the self-bonding of a mass of

substantially pure silicon carbide, a large proportion of which is comminuted to powdered form, the said silicon carbide having been treated to remove the surface impurities which form on the crystal faces of the silicon carbide during its manufacture. 70

4. A silicon carbide resistor having a positive temperature coefficient of resistance formed from the self-bonding of a mass of substantially pure silicon carbide, a large proportion of which is comminuted to a mesh of 200 or finer, the said silicon carbide having been treated to remove the surface impurities which form on the crystal faces of the silicon carbide during its manufacture. 75 80

5. A silicon carbide resistor having a positive temperature coefficient of resistance formed from the self-bonding of a mass of substantially pure silicon carbide, at least 50% of which is in powdered form, the said silicon carbide having been treated to remove the surface impurities which form on the crystal faces of the silicon carbide during its manufacture. 85

6. A silicon carbide resistor having a positive temperature coefficient of resistance formed from the self-bonding of a mass of substantially pure silicon carbide of which between 50 and 80% is in powdered form, the said silicon carbide having been treated to remove the surface impurities which form on the crystal faces of the silicon carbide during its manufacture. 90 95

7. The method of making a silicon carbide resistor having a positive temperature coefficient of resistance which comprises preparing silicon carbide in granular form, mixing therewith between 50 and 80% of powdered silicon carbide, molding a resistor from this mix and then recrystallizing the mix by passing an electric current therethrough, the silicon carbide being first cleaned to remove those mineral impurities which form on the crystals during the manufacture thereof. 100 105

8. The method of making a silicon carbide resistor which comprises reducing commercial silicon carbide to a grain size suitable for use in forming resistors, washing the grain in an acid to remove those mineral impurities which form on the grains during the manufacture of silicon carbide, molding the washed grain to shape to form a resistor, and thereafter securing the resulting article by effecting the recrystallization thereof. 110 115

9. A recrystallized silicon carbide resistor made from silicon carbide grain which has been purified by acid treatment, said resistor having a positive temperature coefficient of electrical resistance over at least a part of its operating range. 120 125

10. A recrystallized silicon carbide resistor made from silicon carbide grain which has been purified by acid and alkali washing, said resistor having a positive temperature 130

coefficient of electrical resistance over at least a part of its operating range.

11. The method of making a silicon carbide resistor having a positive temperature coefficient of electrical resistance over at least a part of its operating range, which comprises preparing commercial silicon carbide grains to a grit size for use in a resistor, treating the prepared grains to remove those surface films which form on the grains in the process of their manufacture, molding the treated grains with a binder, and recrystallizing the formed article while passing an electric current lengthwise through the article.

12. The method of making a silicon carbide resistor having a positive temperature coefficient of electrical resistance over at least a part of its operating range, which comprises the steps of preparing commercial silicon carbide grains to a grit size for use in a resistor, washing the prepared grains in an acid bath, molding the treated grains with a binder, and recrystallizing the formed article while passing an electric current lengthwise through the article.

13. The method of making a silicon carbide resistor having a positive temperature coefficient of electrical resistance over at least a part of its operating range, which comprises preparing commercial silicon carbide grains to a grit size suitable for use in a resistor, treating the grains by washing them in an acid and then in an alkaline bath to remove those surface films which form on the grains in the process of their manufacture, molding the treated grains with a binder, and recrystallizing the formed article while passing an electric current lengthwise through the article.

In testimony whereof we have hereunto set our hands.

JOHN A. BOYER.  
ALMER J. THOMPSON.

45

50

55

60